

## UNITED STATES PATENT OFFICE

1,942,261

## ALLOY

Howard Scott, Wilkinsburg, Pa., assignor to Westinghouse Electric & Manufacturing Company, a corporation of Pennsylvania

No Drawing. Application February 8, 1930  
Serial No. 427,061

## 11 Claims. (Cl. 75—1)

My invention relates to alloys and more particularly to alloys having low coefficients of expansion at ordinary temperatures.

The principal object of my invention is to provide an alloy containing iron, nickel and cobalt that has a low coefficient of expansion.

Another object of my invention is to provide an alloy containing iron, nickel and cobalt that shall have a low, reversible coefficient of expansion over a comparatively wide range of temperatures.

A further object of my invention is to provide an alloy containing iron, nickel, cobalt and carbon in such proportions that the alloy shall have a low coefficient of expansion at normal temperatures, which characteristic will be permanent even though the alloy be subjected to temperatures varying over a considerable range.

Heretofore, an iron-nickel alloy containing approximately 36% nickel has been employed for applications requiring low expansivity at normal temperatures. This alloy is known in the art as Invar and, under ordinary conditions, has an expansivity of .8 to  $2.0 \times 10^{-6}$  per degree centigrade, although a slightly negative expansivity can be conferred upon the best grades by cold working. The necessity for cold working, however, restricts its application because heating the alloy counteracts the decreased expansivity which is obtained by the cold-working process.

I have made the discovery that, if cobalt is substituted for part of the nickel in an alloy, such as Invar, in certain definite proportions, an improved product will be obtained having an approximately zero coefficient of expansion at normal temperatures and a high degree of stability although subjected to severe temperature changes. Experiments clearly demonstrate that my improved alloy is superior to Invar in the manufacture of such articles as pendulums, thermostats, gauges, length standards and tape measures.

It is well known that, if nickel is added in certain proportions to iron, the temperature at which the transformation between the gamma and alpha structures of iron takes place will be reduced below normal temperatures. When the nickel content is approximately 36%, the transformation point is reduced below that of liquid air, and such alloys, accordingly, have a reversible coefficient of expansion over a comparatively wide range of temperatures. An alloy containing about 36% nickel also has the lowest coefficient of expansion of any known iron-nickel alloy. I have found, however, that, if cobalt is

substituted for part of the nickel, the coefficient of expansion of the alloy will be still lower, and the low-expansion characteristic will be stable over substantially the same range of temperatures.

The substitution of cobalt for nickel, however, raises the temperature at which the transformation of the iron from the gamma to the alpha state takes place, but, if the cobalt which is substituted for the nickel is maintained within certain definite proportions, this factor will not adversely affect the commercial value of the alloy because articles manufactured from it will not ordinarily be subjected to temperatures lower than  $-100^{\circ}$  to  $0^{\circ}$  centigrade.

The amount of cobalt that may be substituted for nickel is also dependent upon the amount of carbon and manganese which are present. In my researches, I have found that manganese and carbon are 2.5 and 18 times, respectively, as effective as nickel in reducing the temperature at which the transformation point between gamma and alpha iron takes place, providing the carbon is maintained in solid solution. The amount of carbon which may be maintained in solid solution by the ordinary melting and casting process is limited to approximately 0.3%, although this amount may be increased to over 0.5% by an appropriate heating operation, such as that of heating the alloy to a temperature of  $700^{\circ}$  centigrade or higher and then cooling rapidly.

In practicing my invention, cobalt, iron and nickel, in the proper proportions, are melted together in a suitable furnace, such as an electric furnace. Just before pouring, a small quantity of manganese and silicon are preferably added to render the alloy forgeable, and, in applications requiring a high degree of dimensional stability, the amount of carbon should preferably be maintained below .3%. The alloy may then be cast into ingots in the usual iron or steel molds, after which it may be fabricated in the usual manner, as by forging, or it may be subjected to a hot or cold rolling operation, and the desired articles formed by the usual punching or machining processes.

When neither manganese nor carbon is present, the amount of cobalt that may be substituted for part of the nickel in an alloy containing a nickel-plus-cobalt content of 33% to 38% will range from 2% to 8%. By making such a substitution, the temperature at which the transformation point between gamma and alpha iron takes place will vary between  $-100^{\circ}$  C. and 110

0° C. The presence of carbon in solid solution in my alloy is beneficial because it does not materially affect the expansion characteristics of the alloy, and, since it is 18 times as effective as 5 nickel in reducing the temperature at which the transformation takes place, it permits the substitution of a greater percentage of cobalt for nickel. I have found it highly desirable to have carbon present in amounts ranging up to at 10 least .3% and, for alloys requiring a minimum coefficient of expansion, the maximum amount of carbon that may be retained in solid solution should be present.

Carbon, in the graphitic form, has practically 15 no effect in reducing the transformation point, so that the amount of cobalt that may be substituted for nickel will depend on the carbon which is in solid solution. I do not wish to limit my invention, however, to alloys containing a low 20 percentage of carbon because when iron-nickel-cobalt alloys having a nickel-plus-cobalt content between 33% and 38% are cooled, the carbon either remains in solid solution or separates out in the graphitic form. In certain applications 25 of my improved alloy, it is desirable to prepare articles of a particular shape by casting. In such instances, the addition of carbon improves the casting properties without materially affecting the expansion properties. When such 30 articles are formed, it is desirable, however, to subject the cast article to a heat treatment, to relieve stresses and improve the stability of the alloy, as by heating to approximately 500° C. and then cooling. The amount of carbon that may 35 be added in such cases will depend upon the strength desired in the finished article. Ordinarily, however, not more than 5% should be present.

The addition of manganese is made for the 40 purpose of increasing the forgeability of the alloy. Manganese, however, increases the coefficient of expansion of the alloy, and it is essential that it be maintained as low as possible. For alloys requiring a minimum expansivity, not more than 45 1% should be employed. It will also be understood that other elements which will confer forgeability may be substituted for the manganese, such, for example, as magnesium.

As previously specified, I prefer to substitute 50 cobalt for nickel in as large a proportion as possible consistent with maintaining the temperature of the transformation point below atmospheric temperatures. The following equation indicates the preferable percentages of cobalt that 55 may be employed in an alloy containing a combined cobalt and nickel content of 33% to 38%.

$$\% \text{Co} = 3.9(\% \text{Mn}) + 16(\% \text{C}) + 2\% \text{ to } 8\%$$

In an iron-nickel-cobalt alloy which is substantially free from carbon and manganese and which contains a combined cobalt-nickel content of 36%, 3% of cobalt will raise the temperature of the transformation point to about 60 -100° C. A cobalt content of 8%, in such circumstances, would raise the transformation point to approximately 0° C. In order to produce an alloy of such a type that will have the minimum reversible expansion characteristics at normal temperature, the cobalt content should not exceed 8% and the nickel-plus-cobalt content should not exceed 38%. When carbon and manganese are present, however, the cobalt content may be increased because both carbon and manganese are effective in lowering the temperature at which 70 the transformation point between gamma and 75

alpha iron occurs, so that the total amount of cobalt that may be substituted for the nickel is 2% to 8% plus 3.9 times the percentage of manganese plus 16 times the percentage of carbon, and the temperature at which the transformation takes place when such a substitution is made, will range between -100° C. and 0° C., depending upon the amount of cobalt substituted for the nickel.

In order that the transformation point of the 85 alloy may be safely maintained below normal temperatures and a minimum expansivity obtained over a wide range of temperatures, I prefer an alloy containing a combined nickel-and-cobalt content of 36%, of which amount the cobalt will 90 be equal to 3 plus 3.9 times the percentage of manganese plus 16 times the percentage of carbon. In order to avoid expensive annealing processes, the carbon is preferably maintained at about .3% and the lowest amount of manganese 95 that is effective in rendering the alloy forgeable is approximately .2%, so that the amount of cobalt in such an alloy will be between 8% and 9%, and the nickel content will be between 26% and 27%. An iron-base alloy containing 26.8% 100 nickel, 8.6% cobalt, .3% carbon and .2% manganese has proved very satisfactory. It will be understood that such an alloy may also contain small proportions, say less than 1%, of other elements such as deoxidizers, that do not materially affect its coefficient of expansion or the transformation point, for instance silicon, aluminum or magnesium or two or more of such elements.

If the amount of carbon in solid solution is reduced, it is necessary to reduce the amount of 110 cobalt. For example, the preferred nickel and cobalt content of an alloy substantially free from carbon and containing .2% manganese would be 31.6% and 3.8%, respectively. Such an alloy is 115 preferred in articles requiring a high degree of dimensional stability. If the proportion of manganese in such an alloy is relatively high, for instance, .5%, and .3% of carbon is present, the percentage of the cobalt can be increased to approximately 10%.

While I have described my invention in considerable detail and have given numerous examples, it will be understood that I do not desire to limit myself to the specific details set forth in the foregoing examples, which should be construed as illustrative and not by way of limitation, and, in view of the numerous modifications which may be effected therein without departing from the spirit and scope of my invention, it is desired that only such limitations shall be imposed as are indicated in the appended claims.

I claim as my invention:

1. A low expansion iron-base alloy comprising a combined nickel-and-cobalt content between 125 33% and 38%, and small amounts up to the order of one percent of additional element from the group consisting of carbon and manganese, the amount of cobalt varying from 2% to 8%, the balance of the alloy being substantially iron 140 and the alloy being of reversible, low expansivity below about  $8 \times 10^{-6}$  expansivity.

2. A low expansion iron-base alloy comprising nickel and cobalt, and small amount of carbon in maximum amount of about 0.5%, the nickel-plus-cobalt content varying between 33% and 145 38%, the amount of cobalt present being equal to from 2% to 8% plus 16 times the amount of carbon that is in solid solution, the balance of the alloy being substantially iron and the alloy 150

being of reversible, low expansivity below about  $8 \times 10^{-6}$  expansivity.

3. A low-expansion iron-base alloy comprising nickel, cobalt, small amounts of carbon in a maximum of about 0.5% and small amounts of manganese in a maximum of about one percent, the nickel-plus-cobalt content varying from 33 to 38%, the amount of cobalt being equal to 2% to 8% plus 3.9 times the amount of manganese 5 plus 16 times the amount of carbon in solid solution, the balance of the alloy being substantially iron.

10 4. A low expansion iron-base alloy comprising nickel and cobalt, and small amount of manganese up to 1%, the nickel-plus-cobalt content varying between 33% and 38% and the cobalt content varying between 2% to 8% plus 3.9 times the manganese content, the balance of the alloy being substantially iron and the alloy being 15 reversible, low expansivity below about  $8 \times 10^{-6}$  expansivity.

20 5. A low expansion iron-base alloy comprising nickel, cobalt and .2% to .5% manganese, the nickel-plus-cobalt content varying between 35% and 37% and the amount of cobalt being equal to 2% to 8% plus 3.9 times the amount of manganese, the balance of the alloy being substantially iron and the alloy being of reversible, low expansivity below about  $8 \times 10^{-6}$  25 expansivity.

30 6. A low expansion iron-base alloy comprising nickel, cobalt, and small amount of carbon in maximum amount of about 0.5% and the nickel-plus-cobalt content varying from 35% to 37% of which amount the cobalt will be equal to 2% 35 to 8% plus 16 times the amount of carbon that is in solid solution, the balance of the alloy being substantially iron and the alloy being of reversible, low expansivity below about  $8 \times 10^{-6}$  40 expansivity.

45 7. A low expansion iron-base alloy comprising nickel, cobalt with carbon in maximum amount

of about 0.5%, .2% to .5% manganese, the nickel-plus-cobalt content varying from 35% to 37%, and the cobalt content being equal to 2% to 8% plus 3.9 times the amount of manganese plus 16 times the amount of carbon that is in solid solution, the balance of the alloy being substantially iron and the alloy being of reversible, low expansivity below about  $8 \times 10^{-6}$  expansivity.

85 8. A low-expansion iron-base alloy containing approximately 25 to 32% nickel, 10% to 2% cobalt in accordance with the amount of nickel present, and small amounts of manganese and carbon in maximum amounts of about 1% and 0.5% respectively, the balance of the alloy being substantially iron.

90 9. A low-expansion iron-base alloy containing approximately 25 to 32% nickel, 10% to 2% cobalt and small amounts of manganese and carbon in maximum amounts of about 0.2% and 0.3% respectively, the balance of the alloy being substantially iron.

95 10. A low expansion article of manufacture comprising a ferrous-base alloy containing nickel and cobalt, the cobalt being about eight percent and the nickel-plus-cobalt content of said alloy 100 amounting to 33% to 38% the balance of the alloy being substantially iron and the alloy being of reversible, low expansivity below about  $8 \times 10^{-6}$  expansivity.

105 11. A low expansion iron-base alloy containing nickel, cobalt and small amounts up to the order of one percent of additional element from the group consisting of silicon, aluminum, magnesium, manganese and carbon, the nickel-plus-cobalt content varying between 33% and 38% 110 and the amount of cobalt ranging from about 2% to 10%, the balance of the alloy being substantially iron, and the alloy being of reversible, low expansivity below about  $8 \times 10^{-6}$  115 expansivity.

HOWARD SCOTT.

45

120

50

125

55

130

60

135

65

140

70

145

75

150